

## UNITED STATES PATENT OFFICE.

HARRY CHISLET, OF SCHENECTADY, NEW YORK, ASSIGNOR TO GENERAL ELECTRIC COMPANY, A CORPORATION OF NEW YORK.

## METHOD OF DEPOSITING EMULSIFIED SOLIDS.

No Drawing.

Application filed August 16, 1926. Serial No. 129,647.

The present invention comprises a method of depositing the disperse phase of an emulsion on the surface of a solid, and it is of particular utility for the coating of metal or other objects with water japan, which is an aqueous coating material described in U. S. Patent #1,294,422, issued to Wheeler P. Davey on February 18, 1919.

Heretofore, the coating of solids with water japan has been carried out for commercial purposes either by dipping the object while heated into the emulsion in water of japan-forming materials, which constitutes water japan, or by electrically migrating the emulsified particles of japan-forming materials out of the water and depositing them upon an electrode. Ordinary methods of applying paint, such as brushing, cannot be used advantageously in the case of water japan because the japan is too dilute to get a practical coating by these methods.

In accordance with my invention, I have provided a method of depositing emulsified material on a solid whereby coagulation of the emulsified material (the disperse phase) is produced by an electrolyte and the coagulated material is caused to adhere to the solid surface.

In carrying out my invention, the surface to be coated with japan is provided with a surface film of electrolyte. Preferably an electrolyte in solution is applied which will remain on the surface as a solid upon evaporation of the solvent. For example, the object to be coated may be dipped into an aqueous solution of an alkali, such as sodium or potassium hydroxide. A solution having a concentration of one-half to two per cent of alkali is satisfactory. The object is dried, leaving a thin film of alkali on its surface.

The coated object then is dipped into the emulsion, and the alkali causes the deposition of a layer of the emulsion by the coagu-

lation of the disperse phase adjacent the film coated surface. The coagulated material forms an adherent layer on the surface of the object. Upon withdrawal of the object the layer is baked on as described in the above prior patent. Diffusion of the alkali which goes into solution in the water forming the dispersion medium does no harm. Other electrolytes such as various salts, for example, sodium chloride, may be used, but an alkali is preferred.

The chief advantage of the present method is its cheapness and the ease with which it can be employed under circumstances which make it impracticable to use the special equipment required for the other methods.

What I claim as new and desire to secure by Letters Patent of the United States, is:

1. The method of coating an object with japan from an emulsion of japan and water which consists in dipping the object to be coated into a solution of alkali, drying to remove the solvent, leaving a film of alkali and thereupon dipping said filmed object into said emulsion.

2. The method of depositing a thin layer of japan on an object which consists in depositing a film of an electrolyte on the surface of an object, immersing the coated surface in an emulsion in water of japan-forming materials for a sufficient length of time to cause a deposition of a portion of said materials as an adherent layer on said surface, and upon removal baking said layer.

3. The method of depositing japan from an aqueous emulsion on the surface of an object which consists in coating said object with a film of dry electrolyte, and bringing said filmed surface into contact with said emulsion.

In witness whereof, I have hereunto set my hand this 13th day of August 1926.

HARRY CHISLET.